

# UNITED STATES PATENT OFFICE.

WINFIELD S. POTTER, OF NEW YORK, N. Y., ASSIGNOR TO ALLOY STEEL FORGING COMPANY, OF WILMINGTON, DELAWARE, A CORPORATION OF DELAWARE.

## PRODUCTION OF MANGANESE-STEEL FORGINGS.

1,018,362.

Specification of Letters Patent. Patented Feb. 20, 1912.

No Drawing.

Application filed May 20, 1911. Serial No. 628,437.

*To all whom it may concern:*

Be it known that I, WINFIELD S. POTTER, a citizen of the United States, residing at 30 Church street, in the city, county, and State of New York, have invented certain new and useful Improvements in Production of Manganese-Steel Forgings; and I do hereby declare the following to be a full, clear, and exact description of the invention, such as will enable others skilled in the art to which it appertains to make and use the same.

In the production from manganese steel of heavy forgings or even forgings which have but a moderate thickness or cross-section, the ordinary manner of heating to produce the necessary ductility for the forging operation, followed by rapid forming and water quenching results in certain objectionable characteristics in the final product. For example, should the blank be slowly heated through a critical range lying in the neighborhood of 700° C., the metal will be recrystallized into a coarser structure, and by heating it to a temperature as high, for example, as 1200° C. coarse recrystallization of another character results. So also, unless properly conducted under suitable conditions, the working to finished shape may be of such a character as to involve a reduction and pressure insufficient to satisfactorily deliver the product in the desired fine-grained condition. Furthermore, the forging may, in some instances, be finished so hot that, quenched at the finishing temperature, the steel will have too low an elastic limit and will be liable to distortion in service and will fall below the maximum obtainable resistance to abrasive wear.

My invention is designed to obviate these difficulties and involves so conducting the operation that the metal shall be thoroughly worked or compressed and finished at a suitable temperature and then immediately quenched so that the effects due to the proper working or compression at the appropriate temperature employed shall be fixed in the finished product. This suitable temperature which determines the fixing in the finished products of the effects of the required thorough working or compression will hereinafter be termed the "fixation point". By working or compressing the metal at temperatures below this point (i. e., below 1075° C.) and notably by continuing

the working or compressing until a temperature of about 900° C. is reached, the best results are obtained.

In the practice of my invention, the manganese steel blank from which the forging or forgings are to be produced (as, for instance, forged gears, wheels, forgings for use in railway track work, and other forgings of heavy cross-section which involve considerable reduction or molding of the metal and which therefore require for their formation that the metal shall be in a plastic state so as to be readily worked) is heated to a temperature preferably above 1125° C. until the constituents of the metal are in solution throughout the mass and the metal is in a plastic condition. At this temperature, the blank may be partially formed, to such an extent that the completion of the forming operation can be satisfactorily accomplished at a temperature ranging from 1075° C. (the fixation point) downward to about 720° C. and preferably at about 900° C. which, as hereinbefore stated, is found to give the best results.

After the partial forming at the higher temperature above 1125° C., and before the secondary or final forming is begun, the piece is brought to an equalized temperature throughout, preferably to a temperature of about 900° C. referred to, or to such a temperature as will permit the forming operation to be finished at about 900° C. According to the character of the ultimate product and the use for which it is intended, the piece is then either worked or compressed throughout to finished shape, or is worked or compressed in those portions which are to be subjected to the most severe strains to which constitute the wearing portions as, for instance, the teeth of the gear, the tread portion of a wheel, or the like. The finished shape is then immediately quenched in water, so that the effects of working or compressing the parts that are to be subjected to wear and greater strain are fixed therein.

In some instances, the procedure may be varied, with the production of good results and a satisfactory product obtained for the particular use intended. This is notably the case where the character of the forming operation is such as not to require the maximum ductility in the blank to be formed. Thus, the manganese steel ingot or blank may be heated to a temperature of say,

1175° C. until in a uniform and homogeneous state, and may then be rolled or otherwise formed and, after forming, rapidly cooled so as to produce a steel which retains 5 in the cold state the carbids and other constituents in a state of homogeneous solution throughout the mass. In this condition, the blank may be heated, rapidly through the critical range lying approximately between 10 640° C. and 720° C. and thence upwardly to a temperature preferably not exceeding 1075° C. At the highest temperature to which it is thus brought, it may, if necessary, be held until uniformity of temperature 15 is established throughout the mass. In this instance, also, the temperature for completion of the finishing operation will preferably be about 900° C., and the blank will be subjected to the action of the hammer, 20 the press, or other forming mechanism, and immediately given the intended finished shape. Thereupon, it will be immediately rapidly cooled so as to avoid recrystallization and loss of the fine-grained and stiff 25 condition which has been produced by the sequence of the steps described.

The rapid cooling in the operations hereinbefore described will be effected in any suitable way as, for instance, by quenching 30 with water or by water-spraying, depending on the thickness of section and the finishing temperature, the essential being to cause the metal to cool through a range between 720° C. and about 420° C. at a rate sufficiently 35 rapid to avoid separation of carbids or recrystallization.

It will be found that the quality of the metal in the finished product will correspond to the characteristic features of the 40 operation consisting, as hereinbefore indicated, in bringing the constituents of the metal in the first place into a state of homogeneous solution, and finally completing the working and compression at a temperature 45 so chosen as to impart to the metal the desired stiffness or toughness and high elastic limit.

Although a temperature above 1125° C. has been hereinbefore mentioned as preferable for effecting the solution of the carbids 50 and other soluble compounds of the manganese steel, the production of a manganese steel blank in a uniform austenite or gamma iron condition preparatory to the forging operation may be effected in a longer heating operation at a temperature above the change point at about 1025° C., in accord-

ance with my U. S. Patent No. 975,371, dated November 8, 1910.

What I claim is:

1. The process of producing forgings of manganese steel, which consists in forming the same from a manganese steel blank in a plastic condition and having its constituents in homogeneous solution, and completing 65 the forming operation at a temperature below 1075° C., and finally cooling rapidly, thereby obtaining a product in which the steel has a homogeneous fine-grained structure and a high elastic limit. 70

2. The process of producing forgings of manganese steel, which consists in forming the same from a manganese steel blank in a plastic condition and having its constituents in homogeneous solution, and completing 75 the forming operation at a temperature of about 900° C., and finally rapidly cooling, thereby obtaining a product in which the steel has a homogeneous fine-grained structure and a high elastic limit. 80

3. The process of producing forgings of manganese steel, which consists in forming the same from a manganese steel blank in a plastic condition and having its constituents in homogeneous solution, and completing 85 the forming operation at a temperature below 1075° C. and above 720° C. and finally cooling rapidly, thereby obtaining a product in which the steel has a homogeneous fine-grained structure and a high elastic limit. 90

4. The process of producing forgings of manganese steel, which consists in heating a blank of manganese steel at a temperature above 1125° C., working the metal, completing the forming operation at a temperature 95 below 1075° C., and rapidly cooling.

5. The process of producing forgings of manganese steel, which consists in heating a mass of manganese steel until the carbids have been absorbed, cooling to avoid separation of the carbids, reheating rapidly at temperatures between 640° C. and 720° C., heating further to a temperature sufficient to impart the desired ductility, forming the blank at a temperature below 1075° C. and 100 cooling rapidly to a temperature below 420° C. 105

In testimony whereof I affix my signature, in presence of two witnesses.

WINFIELD S. POTTER.

Witnesses:

JOHN C. PENNIE,  
MINERVA LOBEL.